

(No Model.)

C. T. SNEDEKOR.

INSULATION FOR ELECTRIC CONDUCTORS.

No. 408,901.

Patented Aug. 13, 1889.



Witnesses

G. A. Tauberschmidt

S. B. Whitaker

Inventor  
Charles T. Sneedkor

By his attorney  
Whitelock & Wood

# UNITED STATES PATENT OFFICE.

CHARLES T. SNEDEKOR, OF ST. LOUIS, MISSOURI.

## INSULATION FOR ELECTRIC CONDUCTORS.

SPECIFICATION forming part of Letters Patent No. 408,901, dated August 13, 1889.

Application filed June 21, 1889. Serial No. 315,114. (No model.)

*To all whom it may concern:*

Be it known that I, CHARLES T. SNEDEKOR, a citizen of the United States, residing at St. Louis, in the State of Missouri, have invented 5 certain new and useful Improvements in Insulation for Electric Conductors; and I do hereby declare the following to be a full, clear, and exact description of the invention, such as will enable others skilled in the art to which 10 it appertains to make and use the same.

My invention relates to the insulation of electric conductors and other metallic articles and substances; and it consists in a fire-proof coating or covering, the particular construction of which is set forth in the following 15 description and claims.

Many experiments have been made looking to the attainment of the results accomplished by my construction, but, so far as I am aware, 20 with only partial success, many of the conductors, when insulated in the way proposed, being incapable of bending without cracking or breaking the coating and thus destroying the insulation.

25 By my improvement I am able to produce an insulated cable-wire or other similar conductor which has all the flexibility of the original conductor, and which at the same time is able to resist the action of fire.

30 In order that others may understand the nature of my said invention and the manner of making and using the same, I have illustrated my preferred form of cable in the accompanying drawing, in which is shown an 35 enlarged view of a metallic conductor provided with layers of insulating material, and I will now proceed to describe the same.

The wire, cable, or other conductor to be insulated is first covered with a coating of liquid shellac, and before this is dry a coating 40 or covering is applied to the conductor, consisting of some fibrous material—such as cotton, jute, silk, or other similar substance—which has been saturated in a strong solution 45 of alum. This coating is then allowed to become perfectly dry, after which a liquid glue of any preferred kind is applied, upon which, when hardened, I spread a thick coat of heavy varnish. While this varnish is yet damp a 50 dust is applied, consisting, preferably, of about four parts of powdered or ground glass, one

part powdered alum, and one part powdered asbestos. The conductor is then again covered with a fibrous coating which has been first thoroughly saturated with a composition 55 or paste consisting of linseed-oil, litharge, white lead, ground asbestos, and alum. I again cover this with fibrous material which has first been saturated with a solution of alum and allowed to dry. To this dry fibrous 60 coating I next apply a solution of any of the varnish gums dissolved in linseed-oil, and before this coating hardens there is pressed into it a thin coat of asbestos fiber. When this is perfectly dry and hard, the whole is thor- 65oughly coated with varnish.

While I prefer to use all of the ingredients mentioned in the manner set forth, some of the ingredients and parts mentioned may be omitted and yet good results attained. For 70 instance, the coating of glue may be omitted and the powdered glass may be omitted from the dust coating, and the litharge or white lead may be left out of the composition or paste without any great detriment to the insulation. 75

What I claim, and desire to secure by Letters Patent, is—

1. An insulating-covering for electric conductors and other metallic substances, consisting of a coating of alum-saturated fiber 80 secured to the article to be insulated by shellac, a coat of varnish upon said fiber, a powdered non-inflammable coating upon said varnish, a fibrous coating filled with a paste compound of a mineral substance or substances, 85 a coating of dry alum-saturated fibrous material, an asbestos covering, and an outer coating of varnish, substantially as described.

2. An insulating-covering for electric conductors and other metallic substances, consisting of a coating of alum-saturated fibrous material secured to the article to be insulated by shellac, a coat of varnish upon said fibrous material, a powdered non-inflammable coating upon said varnish, a fibrous coating filled with 95 a paste compound of a mineral substance or substances, a coating of dry alum-saturated fibrous material, a coating of gum and oil, an asbestos covering, and an outer coating of varnish, substantially as described. 100

3. An insulating-covering for electric conductors and other metallic substances, con-

sisting of a coating of alum-saturated fibrous material secured to the article to be insulated by shellac or its equivalent, a coating of glue, a coat of varnish upon the glue when hardened, a coating of non-inflammable substance upon said varnish, a fibrous coating filled with a paste compound of a mineral substance or substances, a coating of dry alum-saturated fibrous material, a coating of gum and oil, an asbestos covering, and an outer coating of varnish, substantially as described.

4. An insulating-covering for electric conductors and other metallic substances, consisting of a coating of alum-saturated fibrous material secured to the article to be insulated by shellac or its equivalent, a coating of glue, a coat of varnish upon the glue when hardened, a non-inflammable coating consisting of a composition of powdered or ground glass, powdered alum and ground asbestos, a fibrous coating filled with a paste compound of a mineral substance or substances, a coating of dry

alum-saturated fibrous material, a coating of gum and oil, an asbestos covering, and an outer coating of varnish, substantially as described. 25

5. An insulating-covering for electric conductors and other metallic substances, consisting of a coating of alum-saturated fibrous material secured to the article to be insulated by shellac or its equivalent, a coating of glue, 30 a coat of varnish upon the glue, a coating of non-inflammable substance or substances, a fibrous coating filled with a paste compound composed of litharge, ground asbestos, alum, and oil, a coating of dry alum-saturated fibrous material, a coating of gum and oil, an asbestos covering, and an outer coating of varnish, substantially as described. 35

In testimony whereof I affix my signature in presence of two witnesses.

CHARLES T. SNEDEKOR.

Witnesses:

L. B. WHITAKER,  
ROBT. H. PAYNE.